

Dec. 2, 1941.

W. SEGUINE ET AL

2,264,338

METALLURGY OF LEAD, TIN, AND OTHER METALS

Filed Aug. 2, 1940



WILLIAM SEGUINE  
FRANK HILLIS

Inventors

334

Chas. Silver  
Attorney

## UNITED STATES PATENT OFFICE

2,264,338

## METALLURGY OF LEAD, TIN, AND OTHER METALS

William Seguine and Frank N. Hillis, Baltimore,  
Md., assignors to The Glidden Company, Cleve-  
land, Ohio, a corporation of Ohio

Application August 2, 1940, Serial No. 350,089

14 Claims. (Cl. 75—21)

This invention relates to the metallurgy of lead and tin and especially to the smelting of certain lead-tin residues existing as lead sulfate and tin oxide and contaminated by small quantities of copper, arsenic and antimony.

Among the objects of this invention is the economical recovery of a lead-tin alloy suitable for the commercial production of solder, type metal and analogous alloys.

A further object of this invention is the economical recovery of lead-tin alloys from low grade residues.

A further object of this invention is the purification of lead-tin alloys from impurities, such as copper and zinc.

A further object of this invention is the economic desulfurization of metalliferous material comprising mainly  $PbSO_4$  and  $SnO_2$ , and including substantial content of powdery material. This invention also comprises the desulfurization of metalliferous material comprising  $PbSO_4$ ,  $SnO_2$ , copper compounds and oxygenated lead compounds of arsenic and antimony and including substantial content of powdery material.

A still further object of this invention is the removal of impurities, such as copper and arsenic, from metalliferous material comprising mainly  $PbSO_4$  and  $SnO_2$  and including substantial content of powdery material.

Other, further and more specific objects of this invention will become readily apparent to persons skilled in the art from a consideration of the following description.

In the treatment of metalliferous powdery material, such as metallurgical fumes and by-products, the lead content exists substantially as lead sulfate. If it is endeavored to smelt this residue, which contains a substantial content of powdery material, substantial losses of valuable metals occur because, in the reduction of these metal compounds with carbonaceous material, lead sulfide and tin sulfide are or may be formed, and such compounds at a high temperature volatilize on account of their respective high vapor pressures.

Further, on account of the fine particle size of these residues, substantial mechanical losses occur in smelting. Accordingly, we have found it economical and expedient to subject these residues to a preliminary treatment prior to smelting and this preliminary treatment, which involves desulfurization and agglomeration, is best accomplished by means of an operation technically termed sintering.

In the operation of sintering, the residues are

mixed with approximately 7 to 9% carbon, usually in the form of coke or coal, together with about 10 to 12% water. This water has the effect of pelleting or balling up the fine residues to such a form that a charge thereof is readily permeable to a blast of air. The charge so prepared is placed upon the grates of a sintering apparatus of the downdraft type, such as exemplified by the well known Dwight Lloyd apparatus, although we do not limit ourselves to this machine in the practice of our invention.

Combustion of the carbon by ignition and induced draft has the effect of bringing the charge to a very high heat so that the lead sulfate content is substantially reduced to lead oxide. This lead oxide, which is readily fusible and which readily combines in part with the tin oxide content, forms thereby a sintered or agglomerated mass which, although somewhat friable, is entirely suitable for reduction to metal in an appropriate furnace such as, for example, a blast furnace.

Such sinter, when mixed with lump coke and flux, is then charged into the blast furnace. The reduced metal or alloy is separated from the slag.

We have found that the impurities in the lead-tin residue are almost quantitatively reduced with the lead and tin, so that the metal alloy of lead and tin contains very substantial amounts of copper, antimony and arsenic. It is necessary, therefore, to remove these impurities by drossing. The economical separation resulting in recovery of valuable metals in this dross is an important feature of our invention. For example, when producing by this process a characteristic lead-tin alloy assaying 25% tin it will usually contain about 1.5% antimony and about 2% arsenic. Also, it will contain varying amount of copper; that is, from 2 to 3%, if the aforesaid lead-tin residue is produced from ordinary zinc fume derived from the smelting of copper ores.

If a lead-tin alloy, such as described, is melted in an appropriate vessel or kettle, and the temperature raised to about 800° F. and then slowly cooled, it will be found that a dross appears upon the surface of the metal. If the contents of the kettle be agitated by a suitable stirrer, the production of this dross will be expedited. However, this dross will contain substantial quantities of entrained alloy. Sawdust is added and stirred into the metal, which operation has the effect of what is known technically as "drying" of the dross. This drying effect is most likely due to the fact that the sawdust on charring decreases

the ability of the molten alloy to wet the dross. Other drying agents may be used.

We have found that this dressing continues down almost to the melting point of the alloy and, if continued carefully, the copper content and arsenic content can be reduced to less than 0.2%. The antimony content, however, does not decrease so much, although we have found that important quantities will pass into the dross.

We have discovered that the dross formed with the progressive cooling of the metal varies very substantially in its copper and arsenic content. We have found that copper passes to the dross in the higher reaches of the cooling curve and that arsenic passes into the dross more substantially as we approach the melting point of the alloy.

Furthermore, we have found that the tin content of the dross rises as the temperature at which the dressing is conducted falls. As a result of these discoveries, we have found it possible to segregate the drosses into portions and prefer in general, for purposes of convenience in manufacture, to produce only two fractions, one of which is a high-copper, low-arsenic dross containing comparatively little tin and second a low-copper, high-arsenic dross with a very substantial tin content.

This segregation of the respective drosses enables us to economically recover the metal content. To effectuate this, we return the high-copper dross to the roasting furnace where the metallurgical zinc fumes are first treated. This dross, when mixed with the original zinc fume, is roasted readily to such a form that the copper content becomes acid-soluble and is recovered substantially as herein later described. The tin contents of the dross at the same time also rejoin the tin content in the metallurgical fumes.

The high-arsenic, high-tin dross is returned to the aforesaid sintering machine. We have found that the arsenic content substantially volatilizes and can be thereby removed from the smelting circuit.

It must be noted that the arsenic content of the original lead-tin fume is present as arseniates of lead, in which form arsenic is not readily volatilized in the sintering machine since it requires considerable energy for its decomposition. However, the arsenic present in the dross exists as arsenide, in which form the arsenic readily passes into a gas. It is, therefore, clear that by the segregation of these drosses we have provided means for satisfactorily removing in an economic manner the copper and the arsenic from the tin-lead alloy.

Also, the removal of antimony is not as simple as the removal of arsenic although we very simply reduce the arsenic content of such metal from say 2% to .25%. The antimony, which may be 1.5% in the crude alloy, can only be reduced to .8%-.1%. However, from the commercial standpoint this is not of importance, because it has been found that about 1% antimony in these alloys is permissible.

The specific metalliferous material comprising  $PbSO_4$ ,  $SnO_2$ , copper compounds and oxygenated lead compounds of arsenic and antimony, for the treatment of which our invention is particularly adapted, is obtained from by-product, zinc fume produced during the smelting of secondary non-ferrous metals.

In the smelting of copper, it is usual to recover copper from ores, concentrates and the like by

first smelting these ores, concentrates, etc., with coke and fluxes in appropriate blast furnaces, forming thereby a compound composed of copper, iron and sulfur which is termed a matte. This matte, while still in a liquid condition, is further treated by the well known Bessemer process whereby the iron and sulfur are removed and finally blister copper is obtained. The blister copper is further refined to pure commercial copper by electrolytic treatment.

Since, in the vicinity of some copper smelters there is available a very large quantity of scrap copper materials, it is customary to treat these scrap materials together with the aforesaid ores and concentrates. Non-metallic scrap, for example, oxidized materials, is customarily charged into the blast furnace, whereas coarse metallics may be placed in the Bessemer converter and so treated. This scrap, however, will almost invariably contain large amounts of zinc, lead and tin, so that in copper smelting it is found that these metals, on account of their volatility and the volatility of their compounds, are fumed out into the blast furnace gases and also into the converter gases. To avoid public nuisance and for economic reasons, it is necessary to cool and filter these gases through appropriate devices, such as woolen bags, electrical precipitators, and the like, so that the smelter may discharge a harmless gas to the atmosphere.

By this means, a fume is collected which will analyze approximately as follows:

|          | Per cent |
|----------|----------|
| Zinc     | 45       |
| Lead     | 15       |
| Tin      | 4        |
| Copper   | 1        |
| Iron     | 0.5      |
| Arsenic  | 0.3      |
| Antimony | 0.3      |
| Chlorine | 1.5      |

In addition, there will be present various indeterminable quantities of organic matter derived from the coke and organic constituents of the smelter charges.

This zinc content exists substantially as zinc oxide, with minor amounts of zinc sulfate and zinc chloride, and is readily extractable from the fume by sulfuric acid. However, when this fume is leached with sulfuric acid, the resulting zinc sulfate is quite impure, containing as it does substantial amounts of zinc chloride and organic matter.

Reference may be had to the accompanying drawing, which shows a flow sheet.

A specific example of carrying out our invention is as follows:

A metallurgical fume as heretofore described and of the above analysis is mixed with 15-25% water and agglomerated into coarse granules, balls and pellets and then roasted at 600-800° C. The organic matter of the fume is consumed and the chloride content is substantially all driven off by volatilization.

The roasted product is then attacked with  $H_2SO_4$  in a dissolving tank and the residue or pulp is separated from the liquor by sedimentation, filtration and/or centrifugal action. The residue is then washed and we prefer to return the wash water to the dissolving tank, where the roasted mass is attacked with  $H_2SO_4$ . The liquor, which is separated from the pulp after the acid treatment, is practically free of chlorides and consists chiefly of  $ZnSO_4$  solution and also small

quantities of the sulfates of Cu, Fe, Cd and Ni. Manganese sulfate is also sometimes found in small quantities. This liquor is now subjected to the usual purification and refining, whereby pure  $ZnSO_4$  solution is obtained. From this pure  $ZnSO_4$  solution pure metallic zinc,  $ZnS$  and/or lithopone may be obtained, of high grade and quality.

The washed residue, consisting chiefly of  $PbSO_4$  and  $SnO_2$  with a small content of copper compounds and oxygenated lead compounds of arsenic and antimony, is dried and then mixed with approximately 7-9% carbon (in the form of coal or coke) together with about 10-12% of water. This wetted material is then agglomerated into coarse granules, balls and pellets, after which it is placed upon the grates of a sintering apparatus of the downdraft type, such as exemplified by the well known Dwight Lloyd apparatus. During this sintering, the lead sulfate content is substantially reduced to lead oxide. This lead oxide, which exists in combination with tin as a sinter, is then mixed with lump coke and a suitable flux and then charged into the blast furnace where it is smelted. The reduced metal or alloy is then separated from the slag.

This reduced metal consisting chiefly as an alloy of lead and tin and containing substantial amounts of copper, antimony and arsenic is then introduced into a dressing kettle together with sawdust, the mass stirred and the temperature thereof raised to about  $800^{\circ} F$ . The molten mass is then slowly cooled and subjected to fractional dressing, preferably 2 fractions. The first fraction which is obtained in the higher reaches of the cooling curve is a high-copper, low-arsenic dross containing comparatively little tin. We prefer to return this fraction to the roaster where it is mixed and treated with the granules, balls and pellets of the metallurgical fume, to which water has been added.

The second fraction, obtained in the lower reaches of the cooling curve, is a low-copper, high-arsenic dross with a very substantial tin content. We prefer to return this fraction to the sintering machine, where it is mixed and treated with the coarse particles, balls and pellets of the residue to which coke has been added. During this treatment, the arsenic content of the dross substantially volatilizes and can be thereby removed from the smelting circuit.

After the fractional dressing, the remaining metal is removed from the dressing kettle and this is a high-grade, purified lead-tin alloy.

The present invention is not limited to the specific details set forth in the foregoing examples which should be construed as illustrative and not by way of limitation, and in view of the numerous modifications which may be effected therein without departing from the spirit and scope of this invention, it is desired that only such limitations be imposed as are indicated in the appended claims.

We claim as our invention:

1. In a process of smelting metalliferous material comprising  $PbSO_4$ ,  $SnO_2$ , copper compounds and oxygenated lead compounds of arsenic and antimony and including a substantial powdery content, mixing said metalliferous material with carbon and water and forming coarse particles thereof, then subjecting the mass of coarse material to sintering under induced draft, whereby  $SO_2$  is driven off, the  $PbSO_4$  is reduced to  $PbO$  and the metalliferous charge is desulfurized and sintered, mixing the resulting desulfurized sinter

with carbon and a flux and smelting same whereby alloy and slag are formed, then removing dross containing copper, arsenic and tin from the molten alloy and then volatilizing the arsenic content from said dross by sintering same with carbon.

2. In a process of smelting metalliferous material comprising mainly  $PbSO_4$  and  $SnO_2$  with small content of copper compounds and oxygenated lead compounds of arsenic and antimony and including a substantial powdery content, mixing said metalliferous material with carbon and water and forming coarse particles thereof, then subjecting the mass of coarse material to sintering under induced draft, whereby  $SO_2$  is driven off, the  $PbSO_4$  is reduced to  $PbO$  and the metalliferous charge is desulfurized and sintered, mixing the resulting desulfurized sinter with carbon and a flux and smelting same whereby alloy and slag are formed, then fractionally removing dross containing copper, arsenic and tin from the molten alloy and then volatilizing the arsenic content from fraction of said dross of high arsenic content by sintering said fraction with carbon.

3. In a process of smelting metalliferous material comprising  $PbSO_4$ ,  $SnO_2$ , copper compounds and oxygenated lead compounds of arsenic and antimony and including a substantial powdery content, mixing said metalliferous material with carbon and water and forming coarse particles thereof, then subjecting the mass of coarse material to sintering under induced draft, whereby  $SO_2$  is driven off, the  $PbSO_4$  is reduced to  $PbO$  and the metalliferous charge is desulfurized and sintered, mixing the resulting desulfurized sinter with carbon and a flux and smelting same whereby alloy and slag are formed, then fractionally removing dross containing copper, arsenic and tin from the molten alloy while the molten metal is cooled and then volatilizing the arsenic content from fraction of said dross of high arsenic content by sintering said fraction with carbon.

4. In a process of smelting metalliferous material comprising mainly  $PbSO_4$  and  $SnO_2$  with small content of copper compounds and oxygenated lead compounds of arsenic and antimony and including a substantial powdery content, mixing said metalliferous material with carbon and water and forming coarse particles thereof, then subjecting the mass of coarse material to sintering under induced draft, whereby  $SO_2$  is driven off, the  $PbSO_4$  is reduced to  $PbO$  and the metalliferous charge is desulfurized and sintered, mixing the resulting desulfurized sinter with carbon and a flux and smelting same whereby alloy and slag are formed, and then fractionally removing dross containing copper, arsenic and tin from the surface of the molten alloy while the molten metal is slowly cooled.

5. In a process of smelting metalliferous material comprising  $PbSO_4$ ,  $SnO_2$ , copper compounds and oxygenated lead compounds of arsenic and antimony and including a substantial powdery content, mixing said metalliferous material with carbon and water and forming coarse particles thereof, then subjecting the mass of coarse material to sintering under induced draft, whereby  $SO_2$  is driven off, the  $PbSO_4$  is reduced to  $PbO$  and the metalliferous charge is desulfurized and sintered, mixing the resulting desulfurized sinter with carbon and a flux and smelting same whereby alloy and slag are formed, adding a drying agent to the molten mass and fractionally re-

moving dross containing copper, arsenic and tin from the molten alloy while the molten metal is cooled.

6. In a process of smelting metalliferous material comprising  $\text{PbSO}_4$ ,  $\text{SnO}_2$ , copper compounds and oxygenated lead compounds of arsenic and antimony and including a substantial powdery content, mixing said metalliferous material with carbon and water and forming coarse particles thereof, then subjecting the mass of coarse material to sintering under induced draft, whereby  $\text{SO}_2$  is driven off, the  $\text{PbSO}_4$  is reduced to  $\text{PbO}$  and the metalliferous charge is desulfurized and sintered, mixing the resulting desulfurized sinter with carbon and a flux and smelting same whereby alloy and slag are formed, adding sawdust to the molten mass and fractionally removing dross containing copper, arsenic and tin from the surface of the molten alloy while the molten metal is slowly cooled.

7. In a process of smelting metalliferous material comprising  $\text{PbSO}_4$ ,  $\text{SnO}_2$ , copper compounds and oxygenated lead compounds of arsenic and antimony and including a substantial powdery content, mixing said metalliferous material with carbon and water and forming coarse particles thereof, then subjecting the mass of coarse material to sintering under induced draft, whereby  $\text{SO}_2$  is driven off, the  $\text{PbSO}_4$  is reduced to  $\text{PbO}$  and the metalliferous charge is desulfurized and sintered, mixing the resulting desulfurized sinter with carbon and a flux and smelting same whereby alloy and slag are formed, and then removing dross containing copper, arsenic and tin from the molten alloy, a fraction of the dross high in copper and low in arsenic and tin being removed at a higher temperature and a fraction of the dross low in copper and high in arsenic and tin being removed at a lower temperature.

8. In a process of smelting metalliferous material comprising mainly  $\text{PbSO}_4$  and  $\text{SnO}_2$  with small content of copper compounds and oxygenated lead compounds of arsenic and antimony and including a substantial powdery content, mixing said metalliferous material with carbon and water and forming coarse particles thereof, then subjecting the mass of coarse material to sintering under induced draft, whereby  $\text{SO}_2$  is driven off, the  $\text{PbSO}_4$  is reduced to  $\text{PbO}$  and the metalliferous charge is desulfurized and sintered, mixing the resulting desulfurized sinter with carbon and a flux and smelting same whereby alloy and slag are formed, then fractionally removing dross containing copper, arsenic and tin from the molten alloy, while the molten mass is cooled, a fraction of the dross high in copper and low in arsenic and tin being removed at a higher temperature and a fraction of the dross low in copper and high in arsenic and tin being removed at a lower temperature, and then sintering the latter fraction with carbon, whereby the arsenic content is volatilized from said latter fraction.

9. In a process of treating powdery material containing organic matter and zinc, lead, tin, cadmium, nickel, copper, iron, arsenic, antimony and chlorine compounds, said process comprising adding water to said powdery material and forming coarse particles thereof, then roasting said coarse particles, extracting the roasted product with acid, mixing the residue after said acid extraction with carbon and water and forming coarse particles thereof, then subjecting the mass of coarse material to sintering under induced draft, whereby  $\text{SO}_2$  is driven off, the  $\text{PbSO}_4$  is

reduced to  $\text{PbO}$  and the metalliferous charge is desulfurized and sintered, mixing the resulting desulfurized sinter with carbon and a flux and smelting same whereby alloy and slag are formed, and then removing dross containing copper, arsenic and tin from the molten alloy, a fraction of the dross high in copper and low in arsenic and tin being removed at a higher temperature, and a fraction of the dross low in copper and high in arsenic and tin being removed at a lower temperature.

10. In a process of treating powdery material containing organic matter and zinc, lead, tin, cadmium, nickel, copper, iron, arsenic, antimony and chlorine compounds, said process comprising adding water to said powdery material and forming coarse particles thereof, then roasting said coarse particles, extracting the roasted product with acid, mixing the residue after said acid extraction with carbon and water and forming coarse particles thereof, then subjecting the mass of coarse material to sintering under induced draft, whereby  $\text{SO}_2$  is driven off, the  $\text{PbSO}_4$  is reduced to  $\text{PbO}$  and the metalliferous charge is desulfurized and sintered, mixing the resulting desulfurized sinter with carbon and a flux and smelting same whereby alloy and slag are formed, then fractionally removing dross containing copper, arsenic and tin from the molten alloy, while the molten mass is cooled, a fraction of the dross high in copper and low in arsenic and tin being removed at a higher temperature and added to coarse particles of said powdery material for roasting and a fraction of the dross low in copper and high in arsenic and tin being removed at a lower temperature and then sintering the latter fraction with carbon, whereby the arsenic content is volatilized from said latter fraction.

11. In a process of treating metallurgical fume containing organic matter and zinc, lead, tin, cadmium, nickel, copper, iron, arsenic, antimony and chlorine compounds, said process comprising adding water to said metallurgical fume and forming coarse particles thereof, then roasting said coarse particles, extracting the roasted product with  $\text{H}_2\text{SO}_4$ , mixing the residue after said acid extraction with carbon and water and forming coarse particles thereof, then subjecting the mass of coarse material to sintering under induced draft, whereby  $\text{SO}_2$  is driven off, the  $\text{PbSO}_4$  is reduced to  $\text{PbO}$  and the metalliferous charge is desulfurized and sintered, mixing the resulting desulfurized sinter with carbon and a flux and smelting same whereby alloy and slag are formed, then fractionally removing dross containing copper, arsenic and tin from the molten alloy, while the molten mass is cooled, a fraction of the dross high in copper and low in arsenic and tin being removed at a higher temperature and added to coarse particles of said metallurgical fume and a fraction of the dross low in copper and high in arsenic and tin being removed at a lower temperature and added to said coarse particles of carbon and residue after said acid extraction for sintering, whereby the arsenic content is volatilized from said latter fraction.

12. In a process of refining arsenical and copperiferous lead-tin alloy, fractionally removing dross containing copper, arsenic and tin from the surface of the molten alloy while the molten metal is slowly cooled, a fraction of the dross high in copper and low in arsenic and tin being removed at a higher temperature and a fraction of the dross low in copper and high in arsenic and tin being removed at a lower tem-

perature, and then sintering the latter fraction with carbon, whereby the arsenic content is volatilized from said latter fraction.

13. In a process of refining arsenical and copperiferous lead-tin alloy, adding a drying agent to the molten alloy and fractionally removing dross containing copper, arsenic and tin from the surface of the molten alloy while the molten metal is slowly cooled, a fraction of the dross high in copper and low in arsenic and tin being removed at a higher temperature and a fraction of the dross low in copper and high in arsenic and tin being removed at a lower temperature, and then sintering the latter fraction with carbon, whereby the arsenic content is volatilized from said latter fraction. 15

14. In a process of refining arsenical and copperiferous lead-tin alloy, adding sawdust to the molten alloy and fractionally removing dross containing copper, arsenic and tin from the surface of the molten alloy while the molten metal is slowly cooled, a fraction of the dross high in copper and low in arsenic and tin being removed at a higher temperature and a fraction of the dross low in copper and high in arsenic and tin being removed at a lower temperature, and then sintering the latter fraction with carbon, whereby the arsenic content is volatilized from said latter fraction. 10

WILLIAM SEGUINE.  
FRANK N. HILLIS.